# EUROPEAN PATENT SPECIFICATION

(11) **EP 3 175 019 B1**
(45) Date of publication and mention of the grant of the patent: **28.11.2018**
(21) Application number: 15742289.0
(22) Date of filing: 28.07.2015
(51) Int. Cl.: C25B 11/04, C25B 1/26

(54) **CATALYTIC COATING AND METHOD OF MANUFACTURING THEREOF**
KATALYTISCHE BESCHICHTUNG UND VERFAHREN ZUR HERSTELLUNG DAVON
REVÊTEMENT CATALYTIQUE ET SON PROCÉDÉ DE FABRICATION

(30) Priority: 28.07.2014 IT MI20141363
(43) Date of publication of application: 07.06.2017
(73) Proprietor: Industrie De Nora S.P.A., 20134 Milano (IT)
(72) Inventor: BONOMETTI, Valentina, I-20134 Milan (IT); CALDERARA, Alice, I-20134 Milan (IT)
(74) Representative: Reitstötter Kinzebach
(86) International application number: PCT/EP2015/067273
(87) International publication number: WO 2016/016243

(56) References cited:
- EP-A1- 2 757 179
- US-A- 3 776 834
- US-A- 3 853 739
- US-A1- 2011 209 992
- CARL-ERIK BOMAN ET AL: "Refinement of the Crystal Structure of Ruthenium Dioxide.", ACTA CHEMICA SCANDINAVICA, vol. 24, 1 January 1970 (1970-01-01), pages 116-122, XP055176446, ISSN: 0904-213X, DOI: 10.3891/acta.chem.scand.24-0116

## Description

### FIELD OF THE INVENTION

The invention relates to a catalytic coating of valve metal articles suitable for use in highly aggressive electrolytic environments, for example in hydrochloric acid electrolysis cells.

### BACKGROUND OF THE INVENTION

Hydrochloric acid electrolysis is an electrochemical process gaining increasing interest at present, being hydrochloric acid the typical by-product of all major industrial processes making use of chlorine: the increase in the production capacity of plants of new conception entails the formation of significant amounts of acid, whose placement on the market presents significant difficulties. The electrolysis of the acid, typically carried out in two-compartment electrolytic cells separated by an ion-exchange membrane, leads to the formation of chlorine at the anode compartment, which can be recycled upstream resulting in a substantially closed cycle of negligible environmental impact. The construction materials of the anodic compartment must be capable of withstanding an aggressive environment combining acidity, humid chlorine and anodic polarisation while retaining a suitable electrical conductivity; for such purpose, valve metals such as titanium, niobium and zirconium are preferably employed, optionally alloyed titanium being the most common example for reasons of cost and ease of machining. Titanium alloys containing nickel, chromium and small amounts of noble metals such as ruthenium and palladium, like the AKOT® alloy commercialised by Kobe Steel, are for instance of widespread use. The anodes whereon the anodic evolution of chlorine is carried out consist for example of a valve metal article such as a titanium alloy substrate coated with a suitable catalyst, typically consisting of a mixture of oxides of titanium and ruthenium, capable of lowering the overvoltage of the anodic discharge of chlorine. The same type of coating is also used to protect from corrosion some components of the anodic compartment not directly involved in the evolution of chlorine, with particular reference to interstitial areas subject to electrolyte stagnation. The lack of a sufficient electrolyte renewal may in fact lead to a local discontinuity of the passivation layer directed at protecting the valve metal, triggering corrosion phenomena, which are the more dangerous the more they are localised in small areas. An example of areas subject to delimiting interstices is given by the peripheral flanges of both the anodic and the cathodic compartment, whereupon sealing gaskets are typically assembled. In the most favourable cases experienced in the industrial practice, titanium alloys coated with catalytic formulations based on oxides of ruthenium and titanium may ensure a continuous operation in a hydrochloric acid electrolysis plant in the range of 24 to 48 months, before corrosion problems leading to deactivation of the anode structure and/or leakage of cell elements in the flange area take place.

EP 2 757179 A1 describes chlorine evolution anodes which, in addition to amorphous ruthenium oxide, may comprise crystalline ruthenium oxide in an intermediate layer or in a catalytic layer. US 3 875 043 A describes a catalytic coating comprising tantalum oxide and ruthenium oxide. US 3,853,739 A describes a coating made from a solid solution of platinum group metal oxides in an amorphous tantalum binder. Carl-Erik Boman et al. describe in Acta Chemica Scandinavica, vol. 24, 1 January 1970, pp. 116-122 the preparation and characterization of crysatls of ruthenium dioxide having a rutile structure. US 2011/0209992 A1 describes an electrode for an electrolysis cell comprising a catalytic layer containing tin, ruthenium, iridium, palladium and niobium oxides using precursor solutions of hydroxyacetochloride complexes of tin, iridium or ruthenium.

For the sake of improving the competitiveness of the industrial hydrochloric acid electrolysis process it is necessary to further increase the useful lifetime of these components.

### SUMMARY OF THE INVENTION

Various aspects of the present invention are set out in the accompanying claims.

Under one aspect, the invention relates to a coated valve metal substrate, having a coating as defined in claim 1. The coating includes a titanium-free catalytic layer and consisting of the mixture of two phases, namely an amorphous phase of Ta₂O₅ in admixture with a tetragonal ditetragonal dipyramidal crystalline phase containing RuO₂, optionally in solid solution with SnO₂. The inventors have in fact observed that titanium -free coatings are more resistant to chloride attack in acidic solution, presumably because titanium oxides - whose function in a combination with ruthenium dioxide is to act as film-forming component - are present as a mixture of crystalline phases including an anatase TiO₂ phase, substantially weaker than the others. The inventors have also observed that mixtures of oxides of tantalum and ruthenium in an amorphous phase do not contribute to solving the problem in a decisive manner, even if completely free from titanium. When, however, the coating is formed from a mixture of RuO₂ in the typical crystalline form similar to rutile (i.e. tetragonal ditetragonal dipyramidal) and Ta₂O₅ in a basically amorphous phase, the stability of the coating to acid attack is greatly increased. As a further advantage, the overvoltage of the coating towards anodic chlorine evolution is surprisingly reduced. The weight ratio between the amorphous phase of Ta₂O₅ and the crystalline phase is between 0.25 and 2.5, which defines the best range of functioning of the invention. In one embodiment, the RuO₂ component in the tetragonal ditetragonal dipyramidal crystalline phase is partially replaced by SnO₂. (cassiterite). The two dioxides of tin and of ruthenium, whose tetragonal ditetragonal dipyramidal crystalline form turns out to be the most stable, are capable of forming solid solutions in any weight ratio; in one embodiment, the Ru to Sn weight ratio in the tetragonal ditetragonal dipyramidal crystalline phase of the coating ranges between 0.5 and 2, which gives the best results in terms of protection of the substrate as well as of catalytic activity of the coating. In one embodiment, the coating comprises two distinct catalytic layers, one as hereinbefore described in direct contact with the valve metal substrate coupled to an outermost one overlaid thereto with a higher content of ruthenium oxide. This can have the advantage of enhancing on one hand the protective function at the substrate surface and on the other hand the catalytic and conductive properties of the outermost layer, as required for example in the case wherein the coating is used for the catalytic activation of an anodic structure whose outer surface is in direct contact with the electrolyte. In one embodiment, the inner catalytic layer has a weight ratio of amorphous Ta₂O₅ phase to RuO₂-containing crystalline phase (optionally including SnO₂) ranging between 0.25 and 2.5 and the outer catalytic layer consists of an amorphous phase of Ta₂O₅ mixed with a tetragonal ditetragonal dipyramidal crystalline phase of RuO₂ with a Ru to Ta weight ratio between 3 and 5. In one embodiment, between the coating as hereinbefore described - in one or two coats - and the substrate there is interposed a further protective pre-layer consisting of a mixture of oxides of titanium and tantalum. This can have the advantage of improving the anchoring of the catalytic layer to the substrate, at the expense of a resistive penalty deriving from the modest electrical conductivity of mixtures of titanium and tantalum oxides. The magnitude of such resistive penalty can be however very limited, provided the pre-layer has a suitably limited thickness. A total loading of titanium and tantalum oxides of 0.6 to 4 g/m² is a suitable value for a pre-layer to be combined with a catalytic layer containing 20 g/m² of total oxides.

In another aspect, the invention relates to a method for the manufacturing of a coated valve metal substrate as hereinbefore described comprising the optional application of a solution of titanium and tantalum compounds, for example TiOCl₂, TiCl₃ and TaCl₅, to a valve metal substrate in one or more coats, with subsequent thermal decomposition after each coat; the application of a solution of compounds of tantalum, ruthenium and optionally tin in one or more coats, with subsequent thermal decomposition after each coat, until obtaining a first catalytic layer; the optional application of a solution of compounds of tantalum and ruthenium upon the first catalytic layer with subsequent thermal decomposition after each coat, until obtaining a second catalytic layer. In one embodiment, the compounds of ruthenium and tin applied in view of the subsequent thermal decomposition are hydroxyacetochloride complexes; this can have the advantage of obtaining more regular and compact layers, having a more homogeneous composition, compared to hydrochloric or other precursors. The thermal decomposition step after each coat can be effected between 350 and 600 °C, depending on the selected precursor compounds. In the case of decomposition of mixtures of precursors consisting of tantalum chloride and hydroxyacetochloride complexes of ruthenium and optionally of tin, thermal decomposition may for example be carried out between 450 and 550 °C.

The following examples are included to demonstrate particular embodiments of the invention, whose practicability has been largely verified in the claimed range of values. It should be appreciated by those of skill in the art that the compositions and techniques disclosed in the examples which follow represent compositions and techniques discovered by the inventors to function well in the practice of the invention; however, those of skill in the art should, in light of the present disclosure, appreciate that many changes can be made in the specific embodiments which are disclosed and still obtain a like or similar result without departing from the scope of the invention.

### EXAMPLE 1

A 1 mm thick AKOT® titanium alloy mesh was degreased with acetone in a ultrasonic bath and etched in 20% HCI at boiling temperature for 15 minutes. The mesh was cut into a plurality of pieces of 10 cm x 10 cm size for the subsequent preparation of electrode samples.

A solution of precursors for the preparation of the protective pre-layer was obtained by mixing 150 g/l of TiOCl₂ and 50 g/l of TaCl₅ in 10% wt. hydrochloric acid.
A first series of catalytic solutions was obtained by mixing 20% by weight RuCl₃ and 50 g/l TaCl₅ in 10% wt. hydrochloric acid according to various proportions.

Solutions of hydroxyacetochloride complexes of Ru (0.9 M) and Sn (1.65 M) were obtained by dissolving the corresponding chlorides in 10% vol. aqueous acetic acid, evaporating the solvent, taking up with 10% aqueous acetic acid with subsequent evaporation of the solvent for two more times, finally dissolving the product again in 10% aqueous acetic acid to obtain the specified concentration.

A second series of catalytic solutions was obtained by mixing the hydroxyacetochloride complexes of Ru and Sn according to various proportions.

Electrode samples were obtained at different formulations with the following procedure:
- a protective pre-layer was applied to the samples cut out of the titanium mesh by brushing the solution containing TiOCl₂ and TaCl₅ precursors in two coats, with subsequent drying at 50 °C for 5 minutes and thermal decomposition treatment at 515 °C for 5 minutes after each coat, until obtaining a deposit of oxides of tantalum and titanium with a loading of about 1 g/m²;
- catalytic layers of various formulations were applied upon the protective pre-layer of the above samples by alternatively applying catalytic solutions of the first or of the second series. The catalytic solutions of the first series were applied by brushing in 8-10 coats and subjected to subsequent drying at 50 °C for 10 minutes and thermal decomposition treatment at 500 °C for 5 minutes after each coat, until obtaining a deposit of oxides of tantalum and ruthenium with a total ruthenium loading of about 20 g/m². At the end of the thermal decomposition process, the electrodes were subjected to a subsequent thermal cycle of 2 hours at 500° C, until obtaining a crystalline tetragonal ditetragonal dipyramidal ruthenium dioxide phase mixed with the amorphous tantalum oxide phase, as verified by means of a subsequent XRD investigation. Some samples of electrodes thus obtained are indicated in Table 1 as RuTa type. The catalytic solutions of the second series have been applied by brushing in 8-10 coats and subjected to subsequent drying at 60 °C for 10 minutes and thermal decomposition treatment at 500 °C for 5 minutes after each coat, until obtaining a deposit of oxides of tantalum, tin and ruthenium with a total ruthenium loading of about 20 g/m². Also in this case, at the end of the thermal decomposition process, the electrodes were subjected to a subsequent thermal cycle of 2 hours at 500 °C, until obtaining a solid solution of ruthenium dioxide and tin dioxide in a crystalline tetragonal ditetragonal dipyramidal phase mixed with the amorphous phase of tantalum oxide, as verified by a subsequent XRD investigation. Some samples of electrodes thus obtained are indicated in Table 1 as RuTaSn type;
- other electrode samples provided with a catalytic coating consisting of two layers were obtained by alternatively applying catalytic solutions of the first or of the second series. The catalytic solutions of the first series were applied by brushing in 6-7 coats and subjected to subsequent drying at 50 °C for 5 minutes and thermal decomposition treatment at 500 °C for 5 minutes after each coat, until obtaining a first deposit of oxides of ruthenium and tantalum; a subsequent solution of the first type with a Ru to Ta weight ratio equal to 4 was subsequently applied by brushing in 2 coats and subjected to the same drying and thermal decomposition cycle after each coat, until obtaining a total ruthenium loading of approximately 20 g/m². At the end of the thermal decomposition process, the electrodes were subjected to a subsequent thermal cycle of 2 hours at 500 °C, until obtaining a crystalline tetragonal ditetragonal dipyramidal phase of ruthenium dioxide mixed with the amorphous phase of tantalum oxide, as verified by a subsequent XRD investigation. Some samples of electrodes thus obtained are indicated in Table 1 as RuTa_TOP type. The catalytic solutions of the second series were applied by brushing in 6-7 coats and subjected to subsequent drying at 60 °C for 5 minutes and thermal decomposition treatment at 500 °C for 10 minutes after each coat, until obtaining a deposit of oxides of tantalum, tin and ruthenium; a deposit of oxides of ruthenium and tantalum, obtained upon brushing in 2 coats of a solution of the first type with a Ru to Ta weight ratio equal to 4, subjected to drying at 50 °C for 5 minutes and thermal decomposition at 500 °C for 10 minutes after each coat, was overlaid thereto, until obtaining a catalytic coating in two layers with a total ruthenium loading of about 20 g/m². At the end of the thermal decomposition process, the electrodes were subjected to a subsequent thermal cycle of 2 hours at 500° C, until obtaining a solid solution of ruthenium dioxide and tin dioxide in a tetragonal ditetragonal dipyramidal crystalline phase mixed with the amorphous phase of tantalum oxide in the inner layer and of a tetragonal ditetragonal dipyramidal ruthenium dioxide crystal phase mixed with the amorphous phase of tantalum oxide in the outer layer, as verified by a subsequent investigation by XRD. Some samples of electrodes thus obtained are indicated in Table 1 as RuTaSn_TOP type.

**Table 1**

| # Sample | Type | Weight composition 1st layer | Weight composition 2nd layer |
|---|---|---|---|
| 1 | RuTa | Ru Ta 25 75 | - |
| 2 | RuTa | Ru Ta 60 40 | - |
| 3 | RuTa | Ru Ta 80 20 | - |
| 4 | RuTaSn | Ru Ta 27 41 Sn 32 | - |
| 5 | RuTaSn | Ru Ta 20 70 Sn 10 | - |
| 6 | RuTaSn | Ru Ta 60 20 Sn 20 | - |
| 7 | RuTa_TOP | Ru Ta 40 60 | Ru Ta 80 20 |
| 8 | RuTa_TOP | Ru Ta 70 30 | Ru Ta 80 20 |
| 9 | RuTaSn_TOP | Ru Ta 20 70 Sn 10 | Ru Ta 80 20 |
| 10 | RuTaSn_TOP | Ru Ta 60 20 Sn 20 | Ru Ta 80 20 |

### COUNTEREXAMPLE 1

A 1 mm thick AKOT® titanium alloy mesh was degreased with acetone in a ultrasonic bath and etched in 20% HCl at boiling temperature for 15 minutes. The mesh was cut into a plurality of pieces of 10 cm x 10 cm size for the subsequent preparation of electrode samples.

A solution of precursors for the preparation of the protective pre-layer was obtained by mixing 150 g/l of TiOCl₂ and 50 g/l of TaCl ₅ in 10% hydrochloric acid.
A series of catalytic solutions was obtained by mixing 20% by weight RuCl₃ and 150 g/l TiOCl₂ in 10% hydrochloric acid according to various proportions.
- a protective pre-layer was applied to the samples cut out of the titanium mesh as in the case of Example 1
- catalytic layers of various formulations were applied on the protective pre-layer of the above samples by brushing the above catalytic solutions in 8-10 coats and subjected to subsequent drying at 50 °C for 5 minutes and thermal decomposition treatment at 500 °C for 5 minutes after each coat, until obtaining a deposit of oxides of ruthenium and titanium with a total ruthenium loading of about 20 g/m². At the end of the thermal decomposition process, the electrodes were subjected to a subsequent thermal cycle of 2 hours at 500 °C. Some samples of electrodes thus obtained are indicated in Table 2 as RuTi type.

**Table 2**

| # Sample | Type | Weight composition |
|---|---|---|
| C1 | RuTi | Ru 25 Ti 75 |
| C2 | RuTi | Ru 60 Ti 40 |
| C3 | RuTi | Ru 80 Ti 20 |

### EXAMPLE 2

The electrode samples shown in the table were subjected to a test of standard potential under anodic evolution of chlorine at the current density of 3 kA/m², in 15% wt. HCl at a temperature of 60 °C. The potential data obtained are reported in Table 3 (SEP). The table shows also the related data of an accelerated lifetime test, expressed in terms of hours of operation before deactivation under anodic evolution of chlorine at the current density of 6 kA/m², in 20% wt. HCl at a temperature of 60 °C, using a zirconium cathode as counterelectrode. The deactivation of the electrode is defined by a 1 V increase in the cell with respect to the initial value.

**Table 3**

| # Sample | SEP (V) | Lifetime (hours) |
|---|---|---|
| 1 | 1.175 | 4020 |
| 2 | 1.168 | 4880 |
| 3 | 1.160 | 4700 |
| 4 | 1.170 | 5770 |
| 5 | 1.173 | 5060 |
| 6 | 1.166 | 5980 |
| 7 | 1.161 | 4550 |
| 8 | 1.154 | 4520 |
| 9 | 1.161 | 5690 |
| 10 | 1.158 | 5540 |
| C1 | 1.190 | 3660 |
| C2 | 1.183 | 3900 |
| C3 | 1.183 | 3280 |

### EXAMPLE 3

Duplicates of electrode samples 2, 6 and C2 were subjected to a corrosion test which simulates the crevice corrosion conditions that can occur on the flanges of electrolysers for the production of chlorine or other occluded zones. A first series of samples was immersed in a known volume of 20% wt. HCl at 45 °C under nitrogen stream, to simulate electrolyte stagnation conditions; a second (control) series was immersed in the same volume of 20% wt. HCl at 40 °C under a stream of oxygen, in order to maintain passivation. In both cases, the concentration of chromium and nickel released from the substrate in the course of 24 hours was detected: for samples 2 and 6, the concentration of both metals in the volume of HCl was less than 2 mg/l, while sample C2 showed concentrations slightly higher than 2 mg/l of Cr and 4 mg/l of Ni under a stream of oxygen, which increased significantly under a stream of nitrogen (up to 6.5 mg/l for nickel).

The test was repeated with another set of samples, confirming a substantial increase in the corrosion resistance for the formulations of the invention.

The foregoing description shall not be intended as limiting the invention, which may be used according to different embodiments without departing from the scopes thereof, and whose extent is solely defined by the appended claims.

Throughout the description and claims of the present application, the term "comprise" and variations thereof such as "comprising" and "comprises" are not intended to exclude the presence of other elements, components or additional process steps. The discussion of documents, acts, materials, devices, articles and the like is included in this specification solely for the purpose of providing a context for the present invention. It is not suggested or represented that any or all of these matters formed part of the prior art base or were common general knowledge in the field relevant to the present invention before the priority date of each claim of this application.

## Claims

1. Coated valve metal substrate having a coating comprising
a titanium-free first catalytic layer consisting of an amorphous phase of Ta₂O₅ in admixture with a tetragonal ditetragonal dipyramidal crystalline phase consisting of either RuO₂ or a solid solution of RuO₂ and SnO₂. said first catalytic layer having a weight ratio of said amorphous phase to said crystalline phase ranging from 0.25 to 2.5 and the Ru to Sn weight ratio in said crystalline phase ranging from 0.5 to 2, and
a second catalytic layer applied externally to said first catalytic layer, said second catalytic layer consisting of an amorphous phase of Ta₂O₅ mixed with a tetragonal ditetragonal dipyramidal crystalline phase of RuO₂ with a Ru to Ta weight ratio ranging from 3 to 5, wherein the content of ruthenium oxide is higher in said second layer than in said first layer.

2. The coated valve metal substrate according to claim 1 comprising a protective pre-layer consisting of a mixture of oxides of titanium and tantalum interposed between the valve metal surface and said first catalytic layer.

3. The coated valve metal substrate according to any one of the preceding claims wherein said substrate is made of titanium or titanium alloy.

4. The use of an anode and/or a flange made from the coated valve metal substrate of any one of claims 1 to 3 in a chlorine-producing electrolyser.

5. The use of claim 4 wherein said electrolyser is a hydrochloric acid electrolyser.

6. Method for manufacturing a coated valve metal substrate according to any one of claims 1 to 3 comprising the following simultaneous or sequential steps:
- optional application of a solution of compounds of titanium and tantalum to a valve metal substrate in one or more coats, with subsequent thermal decomposition after each coat;
- application of a solution of compounds of tantalum, ruthenium and optionally tin in one or more coats, with subsequent thermal decomposition after each coat, until obtaining a first catalytic layer;
- optional application of a solution of compounds of tantalum and ruthenium to said first catalytic layer in one or more coats, with subsequent thermal decomposition after each coat, until obtaining of a second catalytic layer.

7. The method according to claim 6, wherein said compounds of ruthenium and tin are hydroxyacetochloride complexes.

## Patentansprüche

1. Beschichtetes Ventilmetallsubstrat mit einer Beschichtung, umfassend
eine titanfreie erste katalytische Schicht, bestehend aus einer amorphen Phase von Ta₂O₅ unter Beimischung einer tetragonal-ditetragonal-dipyramidalen kristallinen Phase, bestehend entweder aus RuO₂ oder einem Mischkristall aus RuO₂ und SnO₂, wobei die erste katalytische Schicht ein Gewichtsverhältnis der amorphen Phase zu der kristallinen Phase im Bereich von 0,25 bis 2,5 und das Gewichtsverhältnis von Ru zu Sn in der kristallinen Phase im Bereich von 0,5 bis 2 aufweist, und
eine zweite katalytische Schicht, die außen auf die erste katalytische Schicht aufgebracht ist, wobei die zweite katalytische Schicht aus einer amorphen Phase von Ta₂O₅ besteht, gemischt mit einer tetragonal-ditetragonal-dipyramidal-kristallinen Phase von RuO₂ mit einem Gewichtsverhältnis von Ru zu Ta im Bereich von 3 bis 5, wobei der Gehalt an Rutheniumoxid in der zweiten Schicht höher ist als in der ersten Schicht.

2. Beschichtetes Ventilmetallsubstrat gemäß Anspruch 1, umfassend eine schützende Vorschicht, bestehend aus einer Mischung von Oxiden von Titan und Tantal, angeordnet zwischen der Ventilmetalloberfläche und der ersten katalytischen Schicht.

3. Beschichtetes Ventilmetallsubstrat gemäß einem der vorhergehenden Ansprüche, wobei das Substrat aus Titan oder einer Titanlegierung gebildet ist.

4. Verwendung einer Anode und/oder eines Flansches aus dem beschichteten Ventilmetallsubstrat gemäß einem der Ansprüche 1 bis 3 in einem chlorerzeugenden Elektrolyseur.

5. Verwendung gemäß Anspruch 4, wobei der Elektrolyseur ein Salzsäure-Elektrolyseur ist.

6. Verfahren zum Herstellen eines beschichteten Ventilmetallsubstrats gemäß einem der Ansprüche 1 bis 3, umfassend die folgenden gleichzeitigen oder aufeinanderfolgenden Schritte:
- gegebenenfalls Aufbringen einer Lösung von Verbindungen aus Titan und Tantal auf ein Ventilmetallsubstrat in einer oder mehreren Schichten, mit anschließender thermischer Zersetzung nach jeder Schicht;
- Aufbringen einer Lösung von Verbindungen von Tantal, Ruthenium und gegebenenfalls Zinn in einer oder mehreren Schichten, mit anschließender thermischer Zersetzung nach jeder Schicht, bis zum Erhalten einer ersten katalytischen Schicht;
- gegebenenfalls Auftragen einer Lösung von Verbindungen von Tantal und Ruthenium auf die erste katalytische Schicht in einer oder mehreren Schichten, mit anschließender thermischer Zersetzung nach jeder Schicht, bis zum Erhalten einer zweiten katalytischen Schicht.

7. Verfahren gemäß Anspruch 6, wobei die Verbindungen von Ruthenium und Zinn Hydroxyacetochlorid-Komplexe sind.

## Revendications

1. Substrat en métal valve revêtu, comportant un revêtement comprenant :
une première couche catalytique sans titane, consistant en une phase amorphe de Ta₂O₅ en mélange avec une phase cristalline bipyramidale tétragonale ditétragonale consistant en RuO₂ ou en une solution solide de RuO₂ et de SnO₂, ladite première couche catalytique présentant un rapport en poids de ladite phase amorphe à ladite phase cristalline compris dans la plage de 0,25 à 2,5, et le rapport en poids Ru:Sn, dans ladite phase cristalline étant compris dans la plage de 0,5 à 2, et
une seconde couche catalytique appliquée de façon externe sur ladite première couche catalytique, ladite seconde couche catalytique consistant en une phase amorphe de Ta₂O₅ en mélange avec une phase cristalline bipyramidale tétragonale ditétragonale de RuO₂, avec un rapport en poids Ru:Ta compris dans la plage de 3 à 5, la teneur de ladite seconde couche en oxyde de ruthénium étant plus élevée que celle de ladite première couche.

2. Substrat en métal valve revêtu selon la revendication 1, comprenant une précouche protectrice consistant en mélange d'oxydes de titane et de tantale, intercalée entre la surface du métal valve et ladite première couche catalytique.

3. Substrat en métal valve revêtu selon l'une quelconque des revendications précédentes, ledit substrat étant constitué de titane ou d'un alliage de titane.

4. Utilisation d'une anode et/ou d'une bride fabriquée(s) à partir du substrat en métal valve revêtu selon l'une quelconque des revendications 1 à 3 dans un électrolyseur produisant du chlore.

5. Utilisation selon la revendication 4, ledit électrolyseur étant un électrolyseur à l'acide chlorhydrique.

6. Procédé de fabrication d'un substrat en métal valve revêtu selon l'une quelconque des revendications 1 à 3, comprenant les étapes suivantes, simultanées ou successives :
- optionnellement, l'application d'une solution de composés du titane et du tantale sur un substrat en métal valve en une ou plusieurs opérations de revêtement, avec une décomposition thermique subséquente après chaque application d'un revêtement;
- l'application d'une solution de composés du tantale, du ruthénium et en option de l'étain en une ou plusieurs opérations de revêtement, avec décomposition thermique subséquente après chaque application d'un revêtement, jusqu'à l'obtention d'une première couche catalytique ;
- optionnellement, l'application d'une solution de composés du tantale et du ruthénium sur ladite première couche catalytique, en une ou plusieurs opérations de revêtement, avec une décomposition thermique subséquente après chaque application d'un revêtement, jusqu'à l'obtention d'une deuxième couche catalytique.

7. Procédé selon la revendication 6, dans lequel lesdits composés du ruthénium et de l'étain sont des complexes d'hydroxyacétochlorure.
